

Patented Apr. 9, 1929.

1,708,926

# UNITED STATES PATENT OFFICE.

LESTER KIRSCHBRAUN, OF CHICAGO, ILLINOIS, AND ALBERT L. CLAPP, OF DANVERS, MASSACHUSETTS; SAID CLAPP ASSIGNOR TO THE FLINTKOTE COMPANY, OF BOSTON, MASSACHUSETTS, A CORPORATION OF MASSACHUSETTS.

## PAPER AND PROCESS OF MAKING THE SAME.

No Drawing. Application filed February 7, 1921, Serial No. 443,247. Renewed September 24, 1925.

This invention relates to improvements in paper and process of making the same and refers more particularly to the making of waterproof paper in which an adhesive 5 binder, such as asphaltic or bituminous material is incorporated with the paper stock simultaneously with the web forming.

This invention relates to improvements on Letters Patent of the United States issued 10 to Lester Kirschbraun May 6, 1919, No. 1,302,810 and Letters Patent No. 1,536,399, granted May 5, 1925.

Among the salient objects of the invention are to provide a means for precipitating and 15 attaching to the fibres a normally adhesive bituminous binder in emulsified non-adhesive form; to provide a means whereby the fibrous stock is rendered capable of carrying an extremely large amount of the bituminous 20 substance in dispersed form; to provide a process in which the retention of the emulsified bituminous substance during the web-forming operation is promoted or improved; to provide a process in which the bituminous 25 material while in dispersed form is so treated that it attaches itself to the fibrous stock rather than becoming lodged upon the wires and blankets of a paper forming machine; to provide a process in which, through the 30 agency of a bulky precipitant, the dispersed asphalt is enveloped and caused to clot with the fibres in such a manner as to become firmly enmeshed therewith or attached thereto; to provide a process in which the bituminous 35 material in its aqueous vehicle is treated with an agent which causes it to seek contact with the fibrous stock to which the emulsion is added and to cling fixedly with the fibrous material and, in general, to provide a fixing 40 agent by means of which bituminous material may be carried into and by fibrous stock in relatively large quantities and in a non-adhesive state.

Adhesive waterproof materials, such as 45 pitches, asphaltic or other bituminous substances, may be emulsified by heating the same to a temperature above that at which they liquefy, this temperature being ascertained by the melting point of the particular 50 substance to be emulsified, and subsequently combining this liquid adhesive material with an emulsifying agent, such as colloidal clay, in an aqueous vehicle by thoroughly stirring the adhesive substance and emulsifying sus-

pension together. As disclosed in the Letters Patent previously mentioned, an asphaltic emulsion so produced comprises water as the external phase and asphalt as the internal or disperse phase, the particles of asphalt being protected and insulated by clay which 55 is adsorbed upon the surface of the former. It is desirable that the emulsion should contain its asphalt in the finest possible degree of dispersion, it being found in practice that substantially all of the particles will pass 60 through a screen having 40,000 openings to the square inch with many of the finer particles of such size as to show Brownian movement. This process of emulsification is preferably carried on commercially as continuous 65 operation.

It has been the practice heretofore to mix the emulsion so produced with fibrous stock either in the beaters or in the flow box and to run this stock over the paper forming machine 75 to produce a sheet in which the bituminous material is carried and incorporated in the sheet during the web-forming operation. Under such conditions it has been found that the asphaltic particles in the emulsion are 80 more or less loosely associated with the fibrous stock so that when run over the machine considerable quantities of the emulsion released from the stock and flowing out with the back water contact heavily with the wires and 85 blankets, the superficial portions thereof having a tendency to become deposited theron where subjected to pressure and vacuum. In other words, the wet sheet has insufficient 90 attraction for the emulsified asphaltic particles to prevent considerable quantities of the exposed particles from being carried on to the blankets and wires. While, however, the stock is entirely non-adhesive, the association of those non-adhesive particles with the fibrous stock is insufficient to prevent the 95 loss of considerable quantities of asphalt and to permit the maximum service of the blankets and wires. Likewise, as the amount of emulsion in non-adhesive form is increased 100 when producing a sheet with a high degree of saturation, a point is reached when with the increasing amounts of asphalt, the limited carrying capacity of the fibre permits an inordinate loss of emulsified asphalt. The 105 present invention, which involves the use of a fixing agent, as hereinafter described, greatly increases the carrying capacity of

the fibres and causes the emulsified particles to become so strongly attracted and meshed with the stock as to eliminate substantially all tendency for it to deposit on the blanket or wires even under heavy pressure. Thus the formation of the sheet is improved and the ability to run large quantities of the asphalt containing stock over the paper machine is greatly enhanced.

10 The effect of the fixing agent upon the emulsified asphalt particles and the stock is analogous to a clotting action, in that the particles of dispersed asphalt, clay and fibre when in thin aqueous suspension appear aggregated, curdled or flocculated without turbidity of clay and asphalt particles in the water, but with the water between the clotted fibre in a comparatively clear state.

15 In carrying out the present invention, the fibrous stock of desired character is charged to the beater and beaten out in the usual manner. Together with the charge of fibrous stock is added to the beaters a solution of silicate of soda, commonly known as water glass. The percentage of silicate of soda used will, of course, vary with the amount of asphalt to be carried but generally about 1% of concentrated silicate of soda for 10% asphalt to be carried is sufficient. After the 20 stock is beaten out, the asphalt emulsion, prepared as described is pumped to the beaters and a predetermined quantity added to the beaten stock. During the charging of the asphalt emulsion, the beater roll is preferably 25 raised to avoid friction of the knives on the asphalt. The contents of the beater are allowed to circulate until the stock and asphalt are thoroughly mixed together. An excess of aluminum sulphate is then added either in 30 granulated form or in solution sufficient to combine with the sodium silicate and, in addition, to produce the clotting action heretofore described. The amount required can be determined by removing some of the treated stock 35 from the beaters and permitting the water to drain away. Sufficient alum is indicated when the drops of water draining from the stock show clear and free from any signs of turbidity or asphalt emulsion. A sample of 40 this stock will appear to be clotted and when diluted with water in a bottle or test tube will settle rapidly, leaving the water perfectly clear and showing the fibrous stock with its contained asphalt uniformly distributed therethrough. When viewed under the microscope, the particles of asphalt seem to be 45 fixedly attached or clothed upon the fibres with a filmy flocculent envelope enmeshing them with the stock, there being comparatively little of the asphalt unattached.

50 When the stock and emulsion are combined without the use of such a fixing agent, the asphaltic particles are rather loosely associated with the fibre so that when diluted the asphalt particles are seen to be largely float-

ing in the water free from the fibre. When permitted to stand, such stock does not break clear, but produces a turbid suspension which upon settling results in a more or less concentrated layer of asphalt on the fibrous layer. Under the microscope the particles of asphalt seem to be substantially free and detached from the fibrous stock, whereas the stock of the present invention when so viewed shows the asphalt particles surrounded with a bulky precipitate of aluminum silicate, enclosing the bituminous particles and clinging or contacting with the fibers through their feathered-like coatings.

55 An example of the described process is as follows: to 1,000 pounds of stock add 35 to 80 pounds of sodium silicate and after beating thoroughly asphalt is added to an amount of 1,000 pounds. The asphalt, as explained, is in an aqueous emulsion with its contained clay. When this mixture is completed, there is added 100 pounds of aluminum sulphate which, in combination with the sodium silicate, gives the effect heretofore described.

60 In carrying out this process it has been found that in certain instances there is a tendency for the heavy agitation of the beater roll to disturb the clotting effect, both by disrupting the film-like envelopes about the dispersed binder and loosening the binder from the contact with the fibres. In such case, we may treat the emulsified binder by first mixing the emulsion with sodium silicate and then precipitating the sodium silicate with aluminum sulphate, or these reagents may be 65 added to the emulsion in the reverse order and by the addition to the fibrous stock of alkali, such as caustic soda, the treated stock can be maintained in alkaline condition. On the other hand, where aluminum sulphate is 70 in excess, the condition is, of course, slightly acid.

75 The emulsion so treated may be mixed with the fibrous stock in the stuff chest where the agitation is less severe or it may be added to the water withdrawn by the pump from the inside of the cylinder mold, which water is returned to the screens for admixture with the stock. It should be noted that the fixing agent has the effect of fastening the binder and clay upon the fibres while the latter is in a relatively dilute state. It is, of course, well known that it is impractical to incorporate non-fibrous matter with the paper stock without thoroughly beating them together in the beaters even where alum is used as a setting agent, but by means of the fixing agent described the emulsified asphalt may satisfactorily be clotted and carried upon the fibres without beating and even when in a dilute state.

80 While silicate of soda and aluminum sulphate have been mentioned as producing the precipitant giving the desired result, caustic soda may replace sodium silicate, the propor-

tions being so adjusted in such case as to provide an excess of alum for the formation of aluminum hydroxide. We have not as yet been able to ascertain if there is any generic 5 class of substances which have the fixing properties described. While generally the fixing agent is a somewhat gelatinous precipitate, nevertheless all precipitates of this nature do not have the same properties of 10 strongly attracting the asphalt to the fibres. The well known rosin size, for example, which produces with aluminum sulphate an insoluble soap does not have these fixing properties when used in any reasonable quantities. Other substances which have similar 15 fixing properties are produced by the reaction of zinc sulphate and sodium sulphite; tri-sodium phosphate and zinc sulphate; metallic sulphates with sodium sulphide and barium 20 chloride with iron sulphate.

We do not, therefore, intend to limit ourselves to the specific fixing agents mentioned but wish to include all equivalent substances which, when mixed with fibrous stock, show 25 under microscopic examination the properties of fixing and clotting or causing dispersed particles of emulsified bituminous binder or analogous substances to cling to the fibres.

30 The stock produced in accordance with the present invention may be run over any of the commercial paper machines and subjected to a heating and drying operation. The temperature to which the sheet is subjected is 35 sufficient to soften the asphalt particles and cause them to merge, coalesce, flow through the sheet and adhesively unite with the fibres. In some cases it is desirable to dry the sheet at relatively low temperature so as to remove 40 the moisture and cause the asphalt to unite with the fibres but without liquefying the asphalt to coalesce the particles.

We claim as our invention:

1. A method of treating fibrous stock containing a bituminous-pitch type base dispersed in an aqueous medium containing a dispersing agent, comprising causing the emulsified base, while maintaining its dispersed state, to deposit in unaltered state and 45 clot upon the fibrous stock solely by the addition of reacting inorganic substances.

2. A method of treating fibrous stock containing a bituminous-pitch type base dispersed in an aqueous medium containing a dispersing agent, comprising causing the emulsified base, while maintaining its dispersed state, to deposit in unaltered state and 55 clot upon the fibrous stock solely by the addition of an inorganic base and an excess of reacting salt.

3. A method of treating fibrous stock containing a bituminous-pitch type base dispersed in an aqueous medium containing a dispersing agent, comprising causing the 60 emulsified base, while maintaining its dis-

persed state, to deposit in unaltered state and clot upon the fibrous stock by the addition of silicate of soda and a reacting salt to the mixture.

4. A method of treating fibrous stock containing a bituminous-pitch type base dispersed in an aqueous medium containing a dispersing agent, comprising causing the emulsified base, while maintaining its dispersed state, to deposit in unaltered state and 70 clot upon the fibrous stock by the addition of silicate of soda and a metallic sulphate to the mixture.

5. A method of treating fibrous stock for running over a paper machine, comprising 75 mixing the stock with an emulsion comprising a normally adhesive bitumen-pitch type base in a non-adhesive condition in an aqueous medium with an emulsifying agent, and forming bulky aluminum silicate coatings 80 about the particles of emulsified base by the addition of silicate of soda and an excess of aluminum sulphate to the mixture.

6. A method comprising mixing fibrous stock and an aqueous bituminous emulsion in 85 which the bitumen constitutes the dispersed phase, and adding sodium silicate and a metallic sulphate to such mixture to form a flocculent precipitate of metallic silicate surrounding the particles of dispersed bitumen 90 to cause the bitumen to deposit and clot on the fibres.

7. A process of making waterproof paper comprising mixing fibrous stock with bitumen dispersed in an aqueous medium containing 95 an emulsifying agent, causing the emulsified bitumen, while maintaining its dispersed state, to deposit in unaltered state and clot upon the fibrous stock by adding sodium silicate and aluminum sulphate to form 100 aluminum silicate, and subsequently flowing the stock so prepared over a paper-forming machine to remove the water, dry the sheet and cause the bitumen to adhesively unite 105 with the fibres.

8. A process of making waterproof paper comprising mixing fibrous stock with bitumen dispersed in an aqueous medium containing a clay-like emulsifying agent, causing the emulsified bitumen, while maintaining its 110 dispersed stage, to deposit and clot upon the fibrous stock by adding sodium silicate and aluminum sulphate to form aluminum silicate, and subsequently flowing the stock so prepared over a paper-forming machine to 115 remove the water, dry the sheet and cause the bitumen to adhesively unite with the fibres.

9. A process for manufacturing a composite material from pitch and fibrous material, comprising mixing together extremely 120 finely divided pitch and fibrous pulp in an aqueous medium, conditioning the product to permit it to be readily felted into sheets solely by the addition of inorganic substances to 125 the mixture said inorganic substances react- 130

ing with each other, and felting same on a machine of the paper-making type.

10. A process for manufacturing composite material from pitch and fibrous material, comprising mixing together extremely finely divided pitch and fibrous pulp in an aqueous medium, conditioning the stock to permit it to be readily felted into sheets by adding sodium silicate and aluminum sulphate to the mixture whereby the sodium silicate and aluminum sulphate react with each other, and felting same on a machine of the paper-making type.

11. A method which comprises mixing in water, fibrous stock, a dispersion of waterproofing material and silicate of soda, adding a precipitant incapable of reacting with the waterproofing material and running off on a paper machine.

20. 12. A method of conditioning a mixture of fibrous stock and finely divided waterproofing material in an aqueous medium, comprising adding to the mixture an inorganic base, and a salt reacting solely with the inorganic base to cause the particles of waterproofing material to deposit and clot upon the fibrous stock, and then sheeting the mixture on a paper machine.

13. In the method of preparing beater stock, the step which comprises adding a precipitant to an aqueous mixture of fibre, dispersed waterproofing material and silicate of soda, said precipitant being incapable of reacting with the waterproofing material.

35. 14. In the method of preparing beater stock, the step which comprises adding an excess of precipitant to an aqueous mixture of fibre, dispersed waterproofing material and an inorganic base, said precipitant being incapable of reacting with the waterproofing material.

40. 15. In the method of preparing beater stock, the step which comprises adding an excess of precipitant to an aqueous mixture of fibre, dispersed asphalt and an inorganic base, said precipitant being incapable of reacting with the asphalt.

50. 16. A sized fibrous paper-making stock containing dispersed waterproofing particles fixedly attached to and retained on the fibres, substantially wholly by a voluminous flocculent insoluble silicate chemically distinct from the waterproofing particles.

55. 17. A sized fibrous paper-making stock brought to an acidic condition and containing dispersed waterproofing particles fixedly attached to and retained on the fibres substantially wholly by an insoluble inorganic precipitate chemically distinct from the waterproofing particles.

60. 18. A sized fibrous paper-making stock containing dispersed asphalt particles fixedly

attached to and retained on the fibres, substantially wholly by a voluminous flocculent, insoluble silicate uncombined chemically with the waterproofing particles.

19. A sized fibrous paper-making stock brought to an acidic condition and containing dispersed asphalt particles fixedly attached to and retained on the fibres substantially wholly by aluminum silicate.

20. A water-resistant paper product containing asphalt fused onto the fibres thereof, together with aluminum silicate, said product containing also a colloidal emulsifying agent distinct from the aluminum silicate.

21. A water resistant paper product containing 10 to 50% bituminous waterproofing material fused onto the fibres thereof, and fixed thereto with metallic silicate, said product containing also a colloidal emulsifying agent distinct from the silicate.

22. A sized, fibrous paper making stock containing 10 to 50% dispersed asphalt particles fixedly attached to and retained on the fibres substantially wholly by a voluminous, flocculent, insoluble silicate.

23. A sized fibrous paper making stock brought to an acidic condition and containing 10 to 50% dispersed asphalt particles fixedly attached to and retained on the fibres substantially wholly by an insoluble, inorganic precipitate, distinct from the waterproofing particles.

24. A sized fibrous paper making stock containing dispersed waterproofing materials fixedly attached to and retained on the fibres by a voluminous precipitate comprising the reaction product of soluble salts added separately to the stock.

100. 25. A process of making waterproofed paper, which comprises bringing together a batch of fibrous stock and a batch of dispersion of a bituminous base in an aqueous medium, one of said batches containing a precipitant in quantities sufficient to produce an acidic condition in the mixture of fibrous stock and dispersion whereby to cause the bitumen to clot in unaltered state upon the fibers, and running off the mixture on a paper making machine.

105. 26. A process for making fibrous sheet material, which comprises mixing a suspension of beaten fibers and a dispersion comprising solid or semi-solid waterproofing material, water and a protective agent in alkaline medium, adding an excess of acidic substance to the mixture, thus causing dispersed waterproofing material to be carried onto the fiber in unaltered state and subsequently forming 110 into sheets.

LESTER KIRSCHBRAUN.  
ALBERT L. CLAPP.